

April 22, 1930.

H. GEORGE

1,755,953

MANUFACTURE OF TRANSPARENT FUSED PURE SILICA

Filed March 9, 1928



INVENTOR:  
HENRI GEORGE  
by his Attorneys  
Howson and Howson

## UNITED STATES PATENT OFFICE

HENRI GEORGE, OF PARIS, FRANCE, ASSIGNOR TO SOCIETE QUARTZ & SILICE, OF PARIS, FRANCE, A CORPORATION OF FRANCE

## MANUFACTURE OF TRANSPARENT FUSED PURE SILICA

Application filed March 9, 1928, Serial No. 260,455, and in France March 23, 1927.

The present invention has for object an improvement in the methods of manufacture of transparent fused pure silica in which as primary material there is utilized no longer rock crystal, comminuted or not, but compact siliceous rocks employed without grinding up and in the state of as large blocks as possible, for example the special quartzites presenting the following chemical and petrographic characters: high chemical purity, small isometric crystalline elements close-packed without any cement, absence of occluded gases.

The invention relates in particular to the method of fusion of the rocks with a view to the cutting up, the selecting and the shaping of the fused blocks.

When proceeding to the fusion of a large block of natural quartzite presenting the characters previously defined (high chemical purity, small isometric crystalline elements close-packed without any cement, absence of occluded gases), it is easily ascertained that however sound the rock may have appeared, it is comparatively rare that the whole of the block yields after fusion a block of transparent silica not presenting any defect. Thus are found either slightly coloured regions, or flaws ("snows") or bubbles due to local impurities such as a trace of mica. It has been found that these flaws are in general distributed in planes well defined with relation to the primitive rock. The method of fusion constituting the first phase of the present process has for its object to obtain the fusion without deformation of the rock constituting the primary material, in such a way as to avoid bringing the blemished regions into mixture with the sound regions. It will be understood that if such a condition is realized, it will become possible after cooling to divide up the fused mass along the planes containing the flaws in such a way as readily to eliminate the defective regions.

Fusion without deformation of the blocks is rendered possible by the high viscosity of fused silica. The operation consists in arranging the blocks in an electric melting furnace in the midst of a mass of pure siliceous sand, very carefully packed around them, and

in proceeding to the fusion of the whole group of blocks and sand.

The accompanying drawing represents by way of example a melting furnace adapted for this operation.

The metal sheath *a* serves as casing for the furnace and contains the rocks and the sand to be melted. It rests upon a suitable base by the intermediary of trunnions (which are not represented in the figure). A detachable bottom plate *b* closes the furnace at the lower part. This plate is provided with openings allowing the passage of the parts supplying the current to the electrodes. By way of example the furnace represented diagrammatically is a three-phase furnace. The current leads to the electrodes are marked by the arrows 1, 2 and 3. The electrodes themselves are represented at *c* and they are united at the top of the furnace to a piece of graphite *d* serving as neutral point. This arrangement may nevertheless be varied infinitely and the three-phase star-connection is represented in this case only as example. It may be advantageous to provide several electrodes per phase.

In the interior of the cylinder passing through the three electrodes there are arranged the largest blocks of rock *e*. For example with a furnace of 80 centimetres diameter and 1, 5 metres high, there can be arranged in the axis blocks weighing 5 to 10 kilograms. Externally of the cylinder passing through the electrodes, there are arranged smaller blocks. In proportion as the blocks are arranged in the furnace, sand is carefully packed around them. The mounting of the furnace being finished, one proceeds to the fusion and obtains a composite ingot, the contour of which is for example the line *f*. Fusion being completed, the furnace is taken down and the ingot allowed to cool.

The second phase of the process consists in dividing up this ingot by mechanical means of any kind, in order to be able to examine the fused blocks and to divide them up in their turn with elimination of blemished parts, by cutting them up along the planes defined by the flaws. The sound pieces are then examined from the point of view of their trans-

53

65

70

80

85

90

95

100

parency and their optical qualities. The finer ones may be utilized for optical purposes and they are further cut or brought into shape and polished. Those which do not present optical homogeneity are brought into shape or again treated by drawing according to the arrangements of the French Patent No. 585,214, dated 2nd November 1923, and the application for patent filed on 4th May 1926 for "Process and arrangement for the drawing of articles in silica glass or any other vitreous material", or again by hot-stamping according to the application for patent filed on 6th January 1927 for "Process and apparatus for hot-stamping of articles of fused silica and novel articles resulting therefrom", or by mechanical working according to the French Patent No. 601,543, dated 30th October 1924.

What I claim is:

1. A process for the manufacture of transparent, fused, pure silica, consisting in carefully packing a mass of silicious sand around as large blocks as possible of quartzites, said blocks having a high chemical purity, small isometric crystalline elements close packed without any cement and without any occluded gases, in melting said blocks and siliceous sand, and after cooling, in dividing up the composite ingot obtained along the planes containing the flaws or bubbles arising from local impurities, for the purpose described.

2. A process for the manufacture of transparent, fused, pure silica, consisting in carefully packing a mass of silicious sand around as large blocks as possible of quartzites, said blocks having a high chemical purity, small isometric crystalline elements close packed without any cement and without any occluded gases, in melting said blocks and siliceous sand, and after cooling, in dividing up the composite ingot obtained along the planes containing the flaws or bubbles arising from local impurities, and bringing into shape the pieces thus obtained.

In testimony whereof I have signed my name to this specification.

HENRI GEORGE.